

## UNITED STATES PATENT OFFICE

2,187,377

## WEAR RESISTANT ELECTRIC CONTACT

Franz R. Hensel, Indianapolis, Ind., assignor to  
P. R. Mallory & Co. Inc., Indianapolis, Ind., a  
corporation of Delaware

No Drawing. Application September 25, 1937,  
Serial No. 165,767

3 Claims. (Cl. 200—166)

This invention relates to electrical make-and-break contacts.

An object of the invention is to provide an electrical make-and-break contact.

5 Another object of the invention is to improve the characteristics of electric contact elements containing silver.

A further object of the invention is the provision of an electrical make-and-break contact 10 having high wear qualities being produced by means of a special heat treatment.

Other objects of the invention will be apparent from the following description taken in connection with the appended claims.

15 The present invention comprises the combination of elements, methods of manufacture, and the product thereof brought out and exemplified in the disclosure hereinafter set forth, the scope of the invention being indicated in the appended 20 claims.

While a preferred embodiment of the invention is described herein, it is contemplated that considerable variation may be made in the method of procedure and the combination of elements 25 without departing from the spirit of the invention.

For many purposes, it has heretofore been customary to use silver alloys which have desirable electrical characteristics, such as low contact resistance. While such contacts have been found fairly satisfactory, they always had the disadvantage that they are soft and therefore are easily deformed or wear down quickly in service. My invention provides a means to overcome this 30 disadvantage and produce a wear resistant silver base contact material.

My invention consists in using a silver base alloy, containing certain ingredients which have a limited solid solubility in the silver. Furthermore, the solid solubility will change as a function of the temperature. I have found that electrical contact materials of such a structure can be subjected to a simple heat treatment, after which the wear resistance is greatly improved.

40 It is known to use alloys consisting of silver and copper for electrical contacts. The alloys were usually made up in the conventional manner by melting together the ingredients and then forging same down to a size which would allow to 45 either roll the metal into sheet or draw it into wire. I have found that I can take alloys prepared in the above described manner, and produce an increase in hardness heretofore unknown for electrical contact purposes.

50 My preferred heat treatment for improving the

wear resistance of electrical contacts, consists in a quenching operation of the silver base alloy of suitable composition. The temperature from which the alloys are being quenched, usually ranges from 500 degrees C. to just below their melting points, or critical points at which one phase becomes liquid. After this operation, the contact materials are very soft and usually show a minus reading on the Rockwell B scale. The second operation in my preferred heat treatment consists in a drawing at a temperature which is usually below 500 degrees C. In some cases a temperature as low as 200 degrees C. may be used. In general, it can be stated that I can vary the temperature range at which aging proceeds, 10 as long as I vary also the time of aging. Usually at the higher temperature, a shorter time is required to produce the desired results.

The copper-silver alloy, general known as coin silver, containing approximately 10% copper and the balance silver can be heat treated, for instance, by quenching from approximately 750 degrees C. and subsequently aging at 250-300 degrees C. The resulting Rockwell B hardness after such treatment will be 75 Rockwell B or better. In addition, the material can also be cold worked and the hardness still further increased.

I have also found that contact materials which are susceptible to such heat treatment will have an improved electrical conductivity after heat treating. Usually the electrical conductivity is higher, the less material is in solid solution with the silver. The precipitation treatment, which is applied to the contacts in the above described manner, causes the solid solution formed during quenching, to disintegrate and precipitate another phase.

I can regulate the precipitation in such a manner that the precipitated particles are not visible under the microscope, but are very finely and sub-microscopically distributed. Such a very fine and almost homogeneous structure has been proven to be ideally suited for electrical contact purposes. Usually, the best results are obtained in electrical contacts which have only one phase present. If another phase is located, for instance, in the grain boundaries, in the form of large particles, such locations will be attacked during the contact performance and such phenomenon as material transfer will start from these heterogeneous areas. Material transfer can become a very serious obstacle in contact performance and in many cases will determine the life of a contact. By producing the heterogeneous phases in such a finely distributed man-

ner, with the above described heat treatment, I have found that these difficulties can be entirely overcome, and that materials of this nature act as quasi homogeneous.

- 5 I have found that to binary silver copper alloys, also additional metals may be added, without adversely affecting these hardening characteristics. A metal which I have in mind particularly, is cadmium, because the latter produces
- 10 rather desirable contact resistance characteristics in silver base alloys. It is possible to have as much as 16-20% cadmium present and still be able to age harden the silver base alloys. It has been found possible in electrical contact alloys to replace cadmium, either partially or totally, by zinc, and still obtain satisfactory contact performance. In silver alloys of this nature, it is also possible to have up to 5% present of a metal of the iron group or of manganese.
- 15 20 Instead of using pure copper as an age hardening ingredient for silver base electrical contacts, I have found that also intermetallic compounds can be used and I have found that a copper aluminide in silver will produce very effective hardening. With 3% copper aluminide, the hardness can be improved from a minus Rockwell B reading to more than 80 Rockwell B. I have also found that I can substitute for the aluminum one of the elements magnesium, antimony, silicon, palladium, zirconium, titanium, beryllium or chromium.

Since it is possible to vary the elements which are added to the silver base to produce increased hardness by the presence of a highly dispersed phase in a quasi-homogeneous matrix, I do not limit myself to the specific percentages in this disclosure, but use them as illustrative of proportions only and not as limiting proportions.

It is preferred that the dispersed phase be sub-  
40 microscopic in nature and uniformly distributed throughout the matrix of the silver material so

that the resulting composition might be described, as being on the borderline between a solid solution and a heterogeneous mixture, which I describe as a quasi-homogeneous composition.

The electric contact of the present invention can be fabricated into various forms depending upon the uses for which they are required. The contacts may be used whereas silver contacts have been used in the art, as, for example, for relay contact purposes.

While the present invention as to its objects has been described herein as carried out in specific embodiments thereof, it is not desired to be limited thereby, but it is intended to cover the invention broadly within the spirit and scope of the appended claims.

What is claimed is:

1. An age-hardened electric make-and-break contact formed of silver containing copper in amounts not exceeding the solid solubility limits at 750° C. but exceeding the solid solubility limits at 250° C., said contact being characterized by a quasi-homogeneous physical condition wherein there is present a sub-microscopic precipitated phase uniformly distributed and highly dispersed in the silver matrix, said phase consisting predominantly of copper, said contact being further characterized by high hardness and wear resistance imparted thereto by said physical condition.
- 20 25 30 35 40 2. An age-hardened electric make-and-break contact according to claim 1 to which up to 20% of cadmium has been added as a substitute for a corresponding proportion of silver.
3. An age-hardened electric make-and-break contact according to claim 1 to which up to 10% of a material selected from the group consisting of aluminum, zirconium, titanium, palladium, silicon, magnesium and antimony has been added as a substitute for a corresponding proportion of the silver.

FRANZ R. HENSEL.